

# UNITED STATES PATENT OFFICE.

GEORGE C. BAILEY, OF WOODCLIFF-ON-HUDSON, NEW JERSEY, AND FELIX BOETTNER,  
OF NEW YORK, N. Y., ASSIGNEES TO THE BARRETT COMPANY, A CORPORATION  
OF NEW JERSEY.

## TREATMENT OF HIGH-BOILING COAL-TAR DISTILLATES FOR THE PRODUCTION OF RESINOUS PRODUCTS.

1,355,103.

Specification of Letters Patent.

Patented Oct. 5, 1920.

No Drawing.

Application filed October 27, 1919. Serial No. 333,820.

To all whom it may concern:

Be it known that we, (1) GEORGE C. BAILEY, a citizen of the United States, and (2) FELIX BOETTNER, a citizen of Germany, residing at (1) Woodcliff-on-Hudson, N. J., and (2) 170 West 89th St., New York, in the counties of (1) Hudson and (2) New York and States of (1) New Jersey and (2) New York, have invented certain new and useful Improvements in Treatment of High-Boiling Coal-Tar Distillates for the Production of Resinous Products, of which the following is a specification.

This invention relates to the treatment of high boiling coal-tar distillates whereby new products having valuable characteristics are obtained.

In the ordinary distillation of coal-tar to a hard pitch, the highest boiling distillates are the so-called "green oils," which contain the highly useful products anthracene and carbazol, as well as many other bodies less well known. Since the production of anthracene and carbazol entails the formation of much hard pitch, it is desirable that uses for the pitch be developed. Besides the briquetting of coal, one of the uses for this pitch is found in the production of pitch coke, which is useful as a valuable substitute for petroleum coke. It is not economical with the usual type of coal-tar still to run the hard pitch to the coking point, as the high heat necessary would shorten the life of the still very materially, hence a special type of retort is used to convert the hard pitch into a coke, thereby introducing another step in the process of distilling coal tar. During the coking process a high boiling distillate distils or sublimes off from the hard pitch at a high vapor temperature, which distillate may be readily collected. This distillate usually amounts to about two per cent. or more of the hard pitch that is distilled to produce the coke. The actual percentage may vary depending to a certain extent upon the coal-tar pitch charged, the temperature, the time of running the distillation and the character of the retort used. The character of the distillate itself varies to some extent, the same as the other distillates formed during any coal-tar distillation, depending upon the coal-tar source and the other factors. Simi-

lar distillates may be obtained in the high fractions obtained from continuous coal-tar stills as well as from other distillations such as gas circulation, vacuum distillation and others. These distillates are bituminous in character and may properly be referred to as bitumen, within the standard definition of bitumen as given by the American Society for Testing Materials. They are semi-solid to solid at ordinary atmospheric temperatures, boil at high temperatures, and will be referred to in the claims as "semi-solid to solid bitumen of high boiling point obtained from coal tar." This bitumen is often referred to as "pitch resin" by those skilled in this art.

The pitch resin is usually a sticky orange-colored, gummy mass which darkens upon exposure to air. When warmed to slightly above 50° C. it becomes fluid enough to pour from one vessel to another. It possesses few properties in its original state which render it useful for such purposes as an ingredient for varnish, or as resin or gum substitutes. It is not fluid enough for cresoting work and is not hard enough for roofing mixtures. When dissolved in suitable solvents, the solutions darken considerably and from solutions of it in certain solvents crystals may separate.

We have found by experiment that the pitch resin consists in part of solid materials, of truly resinous products, and of certain dark colored, low melting or oily constituents and from our experiments we have developed methods of separating the resinous materials from the solids and oils, and have thereby produced new and useful products.

By experiment we have found that the resin obtained as above described could be distilled completely under a high vacuum and that certain of the distillates were harder than the original resin. We have found that certain solvents will dissolve part of the original pitch resin and leave behind solids which can be crystallized thereby obtaining a dry yellow powder. By combining the two treatments we have worked out a process whereby very transparent hard resins may be obtained.

The following explanation will make the process understood. A quantity of the resin

- is warmed with a solvent, until the mass is quite fluid. For example, if toluene is used as the solvent, the proportions may be about 1000 parts of resin to 120 parts of toluene. 5 The mass is then allowed to cool slowly until it reaches room temperature. It may preferably be cooled by running water or ice water. Upon cooling, the mass becomes somewhat stiff, having an orange color 10 with solid particles therein. The solids may then be removed by a suction filter or a centrifuge or any other convenient and suitable means may be used for separating the solid and liquid constituents. These 15 solids are then washed with a little toluene or other similar solvent and are recovered as a yellow powder which does not darken upon exposure to air, and consists largely or entirely of hydrocarbons melting at about 20 290° C. and over. These solids or crystals sometimes amount to about 8% of the original resin that was treated with the solvent, the amount of solids depending largely upon the nature of the original resin. 25 The filtrate is then distilled to remove the solvent, after which the residue is distilled under a high vacuum and various cuts are made during the distillation. The cuts in the distillation of the filtrate are made 30 at various intervals depending upon the quality and character of the desired products. For example, the solvent is first regained which is re-used in another extraction. Later, up to about 20 C. under an 35 absolute pressure of 8 mm. a heavy oil is obtained which does not solidify and may be returned to the creosote oils. From 220° to about 275° yellowish greases are obtained. From about 275° to about 400° C. under the 40 above absolute pressure transparent red resins are obtained varying in degree of hardness as the temperature increases. These resins may be redistilled if the first distillation does not give suitable products. The 45 hardest resin may melt at 75° C. to 100° by the same empirical methods as used to test the softening point of pitches. This resin is transparent and does not discolor upon standing exposed to air and light. 50 Furthermore a vacuum distillation may be made on the resin as received from the coking retorts and the several cuts washed with suitable solvents and these solutions again distilled or the various cuts from the 55 vacuum distillation may be utilized as they are received from the vacuum still.
- By any of these processes resinous materials may be obtained which are quite hard and possess little tendency to change color upon long standing. The transparent red resins have melting points of a range as wide or wider than from about 40° C. to 100° C. depending upon the temperature at which the cuts are made. These resins are com-
- plex mixtures probably of substances not yet identified chemically.
- Samples of these transparent red resins have been found to contain about 92.2% carbon, 4.6% hydrogen and traces of nitrogen and sulfur. The specific gravity is about 1.256 at 15.5° C. The resinous material is soluble in the ordinary coal tar solvents, chloroform, carbon tetrachlorid, linseed oil, cotton seed oil and others, and partly soluble in methyl alcohol, ethyl alcohol, glacial acetic acid, petroleum naphthas, and ether. 75
- The harder distillates flux when melted carefully with sulfur, para-coumarone or para-indene resins, halowax resins, rosin, montane wax, carnauba wax, etc. 80
- These resins may be utilized in varnish mixtures, rubber compounding, water proofing mixtures and as a substitute for various waxes and resins. 85
- Claims:
1. The herein described process which comprises extracting with a solvent, a semi-solid to solid bitumen of high boiling point obtained from coal tar, separating the solution, removing the solvent from the solution, and distilling the residue under vacuum. 90
  2. The herein described process which comprises extracting a semi-solid to solid bitumen of high boiling point obtained from coal tar with a solvent, filtering, distilling the solvent from the filtrate, and distilling the residue under vacuum. 95
  3. The herein described process which comprises extracting with a solvent, a semi-solid to solid bitumen of high boiling point obtained from coal tar, filtering, distilling the solvent from the filtrate, distilling the residue under vacuum and separating the vacuum distillate into fractions having different boiling points. 100
  4. The herein described process which comprises extracting with a solvent a semi-solid to solid bitumen of high boiling point obtained from coal tar, filtering, distilling the solvent from the filtrate, distilling the residue under vacuum, separating the distillate into fractions having different boiling points and redistilling one or more of said fractions under vacuum. 110
  5. A transparent, red resin derived from a semi-solid to solid bitumen of high boiling point obtained from coal tar which does not darken upon exposure to air and light and which can be distilled under vacuum without substantial decomposition. 115
  6. A transparent red resin derived from a semi-solid to solid bitumen of high boiling point obtained from coal tar which melts above 40° C. and which can be distilled under vacuum without substantial decomposition. 120
  7. A transparent red resin derived from a semi-solid to solid bitumen of high boiling

point obtained from coal tar and containing carbon and hydrogen in substantially the proportion of 20 to 1 and which can be distilled under vacuum without substantial de-  
5 composition.

8. A hard, transparent, red resin derived from a semi-solid to solid bitumen of high boiling point obtained from coal tar, which does not darken upon exposure to air and  
10 light, having a melting point above 40° C.

containing carbon and hydrogen in substantially the proportion of 20 to 1, and being partly soluble in petroleum naphthas and which can be distilled under vacuum without substantial decomposition.

In testimony whereof we affix our signatures.

GEORGE C. BAILEY.  
FELIX BOETTNER.

It is hereby certified that in Letters Patent No. 1,355,103, granted October 5, 1920, upon the application of George C. Bailey, of Woodcliff-on-Hudson, New Jersey, and Felix Boettner, of New York, N. Y., for an improvement in "Treatment of High-Boiling Coal-Tar Distillates for the Production of Resinous Products," an error appears in the printed specification requiring correction as follows: Page 2, line 34, for "about 20 C." read *about 220° C.*; and that the said Letters Patent should be read with this correction therein that the same may conform to the record of the case in the Patent Office.

Signed and sealed this 30th day of November, A. D., 1920.

[SEAL.]

L. B. MANN,

*Acting Commissioner of Patents.*

Cl. 134—26.